

1

3,399,259

## METHOD FOR PRODUCING BICOMPONENT POLYPROPYLENE FILAMENTS

John Raymond Brayford, Harrogate, England, assignor to Imperial Chemical Industries Limited, London, England, a corporation of Great Britain  
 No Drawing. Filed Apr. 7, 1966, Ser. No. 540,852  
 Claims priority, application Great Britain, Apr. 20, 1965,  
 16,543/65  
 8 Claims. (Cl. 264—168)

### ABSTRACT OF THE DISCLOSURE

Self-crimping bicomponent polypropylene filaments are made by conjugate melt spinning two different polypropylene polymers in side-by-side or sheath-core relationship and subsequently relaxing the filaments. The polymers have the same intrinsic viscosity but different molecular-weight distributions. Enhanced crimp is effected by drawing the filaments.

### DISCLOSURE

This invention relates to a process for the production of self-crimping polypropylene filaments or filamentary yarn.

It is known, from British patent specification No. 805,033 to produce filaments from at least two chemically different synthetic polymers by a melt-spinning process wherein the molten polymers are fed separately to the shaping orifices and form filaments having the two polymers distributed non-uniformly across the cross-sections of the filaments, the non-uniformity giving rise to an inherent crimping potentiality in the filaments.

It is also known, from British patent specification No. 979,083 to produce spontaneously crimping polyolefine filaments from two polyolefine components of different viscosity arranged in side-by-side relationship along the length of the filaments.

We have now found that self-crimping polypropylene filaments or filamentary yarn may be produced without this viscosity difference or with a substantially reduced viscosity difference between the two polypropylene components.

According to the present invention we provide a process for the production of self-crimping polypropylene filaments wherein composite filaments having two different propylene polymers distributed along the length of the filaments as distinct components in side-by-side or sheath-core relationship are produced by conjugate melt spinning of two propylene polymers followed subsequently by relaxation of tension in the filaments, characterised in that the two polymers have substantially the same intrinsic viscosity but different molecular weight distributions. We prefer that at least one of said polymers has a dispersion coefficient, Q, as hereinafter defined, of at least 6.5 and that the difference between the Q values of the components should be at least 0.5 for an adequate crimping effect to be obtained.

Filaments or filamentary yarn according to the invention are described as self-crimping for upon release of the tension applied to them during melt-spinning or the subsequent cold-drawing step they contract and take-up a helically crimped form. The tension may be maintained in the filaments between and subsequent to these processes by, for example, winding the filaments or filamentary yarn on to bobbins and then released at an appropriate stage in the subsequent textile processing. Thus, self-crimped staple fibres may be produced by cutting an uncrimped yarn or tow into staple lengths while allowing relaxation to take place. Alternatively the filamentary yarn may be subjected to a mechanical crimping process before release-

2

ing the tension to impede the self-crimping effect sufficiently to facilitate subsequent textile processing.

The substantial absence of mechanical restraint during relaxation will lead to the maximum crimping effect. However in some uses to which the crimped fibres or filaments are put it is desirable to control the extent of crimping achieved as the maximum crimping effect may lead to an undesirable harshness of handle in the resultant yarn or fabric.

Although self-crimping filaments or filamentary yarns produced as in this invention may show the self-crimping effect in the as-spun condition, the effect is much enhanced by drawing the as-spun filaments, preferably to more than twice but not more than about four times their original length at a temperature not exceeding about 100° C.

We have found that the degree of crimping effect obtained upon relaxation may be controlled independently of the composition of the composite fibres by regulating the temperature of the snubbing surface (pin or roll) upon which drawing is effected. As the temperature of the snubbing surface is increased so the crimping effect obtained is decreased until at about 100° C. little crimping is achieved. Thus, for example by drawing composite filaments, the components of which have dispersion coefficients of 8.4 and 4.7 and the same viscosity, 1.55, at a draw ratio of 3.5:1 we obtained the following results for percentage crimp under a load of 0.5 mg./denier as the temperature of the snubbing surface, in this case a heated feed roll, was increased.

| Feed roll, temp. ° C. | Percent crimp at 0.5 mg./den. |
|-----------------------|-------------------------------|
| 55                    | 58                            |
| 65                    | 55                            |
| 75                    | 41                            |
| 85                    | 17                            |

It is preferred to stabilise the helical form of the self-crimped fibres by a heat treatment in the relaxed state at a temperature of about 100–140° C. Some increase of the self-crimping effect may accompany stabilisation of the crimp by the heat treatment.

Several forms of melt-spinning apparatus for conjugate spinning of side-by-side or sheath-core composite filaments are known, as for example, British patent specifications 953,379 and 972,932 and such equipment may be used to form composite polypropylene filaments according to the invention. The terms side-by-side and sheath-core refer to the relationship of the two components in the individual filaments and the term conjugate spinning refers to the production of such composite filaments.

The dispersion coefficient, Q, which is an expression of the molecular weight distribution of a propylene polymer, is the ratio of weight average molecular weight,  $\bar{M}_w$ , to number average molecular weight,  $\bar{M}_n$ . We have determined the Q values of propylene polymers comprising the conjugate filaments from measurements of  $\bar{M}_w$  and  $\bar{M}_n$  by, respectively, light scattering and membrane osmometry techniques which are described in detail hereinafter, using the component polymers as supplied to the conjugate melt spinning apparatus as it is impossible to separate the components of the spun conjugate filaments. Control tests wherein individual propylene polymers are melt spun under conditions identical to those used in the conjugate melt spinning process show that no degradation or change in viscosity or molecular weight distribution is incurred during melt spinning.

### DETERMINATION OF $\bar{M}_w$

For this determination we have used a photo-gonio difusometer Model 42,000 of the Societe Francais d'Instruments de Control et d'Analyse (SOFICA).

Light scattering measurements were carried out at 130°

C. using unpolarised light of wave-length 5461 Å, the light scattering cells being immersed in a temperature controlled oil bath filled with silicone oil. The solvent used for these measurements was  $\alpha$ -chloronaphthalene (British Drug Houses) which was dried and re-distilled under reduced pressure before use, 0.1% w/v. of a phenolic antioxidant then being added to stabilise the distilled material. Solutions of the polymer under test containing 0.1, 0.2, 0.3, 0.4 and 0.5% w/v. were prepared at 130° C. in calibrated 25 ml. flasks. The solutions and the solvent blank used in each measurement were carefully clarified by filtering at 130° C. through a sintered glass filter, to remove all traces of dust etc.

Ten ml. portions of the clean polymer solutions and the solvent blanks were used, measurements being taken at scattering angles of 30–150° (in eleven steps) to the incident beam. Between the measurements for each solution the intensity of the incident beam of light was checked for constancy against the reading at 90° for a standard diffusor.

The instrument was calibrated with benzene and the instrument constant checked against a standard polystyrene specimen of known molecular weight (National Bureau of Standards No. 706,  $\overline{M}_w=258,000$ ). The molecular weight of the standard was calculated using the accepted value of the Rayleigh ratio of benzene,  $16.3 \times 10^{-6}$ , and  $\overline{M}_w$  was found to be 256,000. Benzene was thereafter used as a standard for converting the photomultiplier reading to the absolute scattering intensity by the equation

$$R_\theta = R_b \left[ \frac{\sin \theta}{1 + \cos^2 \theta} \right] \left[ \frac{I_\theta}{I_b} \right] \left[ \frac{\eta}{\eta_b} \right]^2 = R_b \left[ \frac{\alpha I_\theta}{I_b} \right] \left[ \frac{\eta}{\eta_b} \right]^2 \quad (1)$$

where

$$\alpha = \left[ \frac{\sin \theta}{1 + \cos^2 \theta} \right]$$

where  $R_\theta$  is the Rayleigh ratio of the solution (corrected for solvent scattering) at any angle  $\theta$ ,  $R_b$  is the Rayleigh ratio of pure benzene,  $I_\theta$  is the instrument galvanometer deflection for the solution in excess of that of the solvent,  $I_b$  is the galvanometer reading for pure benzene,

$$\left[ \frac{\eta}{\eta_b} \right]^2$$

is the square of the ratio of the refractive indices of the solution to that of benzene.  $\sin \theta$  and  $(1 + \cos^2 \theta)$  are correction factors for the volume of scattering at angle  $\theta$  and the use of unpolarised light respectively.

The usual light scattering equation is

$$\left[ \frac{KC}{R_\theta} \right]_{C=0, \theta=0} = \frac{1}{\overline{M}_w}$$

where

$$K = \frac{2\pi^2 (\eta d\eta/dC)^2}{N \lambda^4}$$

whence by substituting Equation 1 in Equation 2

$$\frac{2\pi^2 \eta_b^2}{N \lambda^4 R_b} \left[ \frac{d\eta}{dC} \right]^2 [I_b] \left[ \frac{C}{\alpha I_\theta} \right]_{C=0, \theta=0} = \frac{1}{\overline{M}_w}$$

where  $\lambda=5461$  Å,  $C$ =concentration, g./ml.,  $N$ =Avogadro's Number and

$$\alpha = \frac{\sin \theta}{1 + \cos^2 \theta}$$

Using the accepted values for the constants we have

$$0.506 \left[ \frac{d\eta}{dC} \right]^2 [I_b] \left[ \frac{C}{\alpha I_\theta} \right]_{C=0, \theta=0} = \frac{1}{\overline{M}_w}$$

For polypropylene in  $\alpha$ -chloronaphthalene at 130° C. and  $\lambda=5461$  Å,  $d\eta/dC=-0.189$  ml./gm. Using this and set-

ting  $I_b=1.32 I_g$  (where  $I_g$  is the scattering intensity of the standard diffusor) we have

$$\overline{M}_w = \frac{73.046}{I_g \left[ \frac{C}{\alpha I_\theta} \right]_{C=0, \theta=0}}$$

In accordance with the last equation Zimm plots were obtained by plotting

$$\left[ \frac{C}{\alpha I_\theta} \right]$$

against  $(\sin \theta/2 + 50)$  C. The term 50 C. is a geometric one to give a good spread of the 55 points contained in each Zimm plot. The extrapolated lines  $C=0$  and  $\theta=0$  should intercept the ordinate at the same point

$$\left[ \frac{C}{\alpha I_\theta} \right]_{C=0, \theta=0}$$

which then gives  $=w$  provided the  $I_g$  value for the measurement is known.

The Zimm plots were only accepted if the lines of points of equal concentration were straight; curved lines indicated inadequate filtering. Repeat measurement on several polymers degraded and undegraded, showed that the accuracy of  $\overline{M}_w$  determination was  $\pm 5000$  units.

#### DETERMINATION OF $\overline{M}_n$

For this determination we have used a high speed osmometer made by Dohrman Instrument Co. to a Shell Development Corporation design, equipped with an "ultracella allerfeinst" membrane made by Membranfilter Gesellschaft, Göttingen.

The membrane was conditioned by immersion for not less than 6 hours in the following sequence of solvent mixtures; water, water/ethanol, ethanol, ethanol/acetone, acetone, acetone/methyl ethyl ketone (MEK) MEK, MEK/toluene, toluene, toluene/decalin and decalin. The membrane was then conditioned for high temperatures by first of all securing it in position in the osmometer and filling the solvent and solution compartments with solvent. The temperature in the osmometer was then raised by 30° C. steps until a temperature of 120° C. was reached allowing 8 hours conditioning at each temperature. The solvent used for the measurements, decalin, was vacuum distilled prior to use and oxidation was inhibited by the addition of 0.1% w/v. of a phenolic antioxidant.

Polymer solutions (with a concentration chosen so as to give a pressure head of at least 1.2 cm. of solvent) were prepared at 130° C. in pre-calibrated volumetric flasks and the solutions so prepared were filtered, prior to injection into the osmometer, at 130° C. through two thicknesses of 0.8  $\mu$  Millipore membrane filters (Millipore Corporation of America). The injected solutions were allowed 5 minutes to equilibrate in a pre-heater in the osmometer before being allowed to enter the solution compartment wherein a further 10 minutes equilibration time was allowed.

The instrument zero was established by repeatedly filling the solution compartment with solvent and measuring the pressure head each time on the manometer servo read-out dial, the instrument zero being taken as satisfactory when three readings agreed to within  $\pm 0.01$  cm. of solvent. The sample outlet was then closed and the equilibrium pressure reading was taken after about 40 minutes. The process was then repeated for another portion of the same solution, whereafter the instrument zero was re-established in the foregoing manner. As solute diffusion was always found to be present, the initial and final instrument values did not agree and the difference in these readings was used to correct the final solution concentration reading for diffusion.

The pressure readings obtained from this instrument are for the solvent at approximately 20–25° C., there-

fore the osmotic pressure  $\pi$  is given by  $(h-h\theta)\rho$  where

$h\theta$ =solvent zero in cms.

$h$ =solution zero in cms.

$\rho$ =density of solvent at 25° C.

The osmotic pressure readings obtained are then plotted as  $\pi/c$  against  $C$ , where  $C$  is the concentration of solute in gm. per 100 ml. The value of  $\bar{M}_n$  is found by extrapolating this graph to zero concentration from the intercept,  $(\pi/C) C=0$  by means of the following equation

$$(\pi/C)_{C=0} = \frac{RT}{\bar{M}_n}$$

where  $R$  is the gas constant and  $T$  is the absolute temperature.

For many purposes a shortened method of measurement is quite satisfactory. Thus instead of measuring the osmotic pressure for a number of polymer solutions of different concentrations and extrapolating the results to zero concentration we have used a single very dilute solution measurement and used this value as a close approximation for  $(\pi/C) C=0$  as we have found that the values so obtained agree with the values by extrapolation of a number of polymer solutions within 3%. Values obtained by the shortened method were therefore increased by a factor of 3% to give a close estimate of  $\bar{M}_n$ . The accuracy of determination is approximately  $\pm 750$  molecular weight units.

Polymers having different molecular weight distributions may be produced in several ways. Thus thermal degradation of polypropylene from a higher to a lower viscosity will cause a narrowing of the molecular weight distribution, the product then being used as one component of a composite filament, the other component being, for example, a polymer which has been subjected to a lower degree of degradation. Alternatively a polymer

manner in which it may be performed. As the force with which self crimping occurs has an effect upon the degree of crimping attained we give in these examples the degree of crimp achieved by (a) substantially free relaxation (0.01 mg./denier) and (b) under a load of 0.5 mg./denier, which is the order of the resistance to relaxation in a loosely twisted multifilamentary or staple fibre yarn such as would be used for example for hand knitting purposes. In order to measure the crimping effect under a specified load we wind small hanks (100 cm. long) of filamentary yarn around a 10 cm. "Perspex" (Regd. Trade Mark) rectangular former, remove the hanks, suspend therefrom an appropriate lead, heat treat in an air oven for 10 minutes at 135° C. and then measure the contracted length of the unwound hank with the load removed ( $L_1$ ) and the length ( $L_2$ ) of the unwound hank with the crimps just removed by extension. The percentage crimp obtained is then expressed as

$$\frac{L_2 - L_1}{L_2} \times 100$$

#### EXAMPLES 1-7

Conjugate melt spinning apparatus, having means for separately supplying two molten polymers to a spinneret 25 at independently controllable rates, is used to produce composite filaments from seven pairs of propylene polymers each pair having the same intrinsic viscosity but different molecular weight distribution and equal proportions of each component. The component polymers 30 join at the spinneret orifices to produce composite filaments of the side-by-side type. The spinnerets used have 24 to 60 orifices of 0.020 inch (0.051 cm.) diameter as noted hereinafter and in all cases except two (Examples 6 and 8) the denier per filaments of the spun filamentary yarns was 35 15. In Examples 6 and 8 the spun denier per filament was 20. Other spinning conditions and additive substances present in the polymers are given in the following table.

| Example No. | Intrinsic viscosity | Q values | No. of orifices | Spinneret temp., °C. | Wind-up speed m./min. | Additives                     |
|-------------|---------------------|----------|-----------------|----------------------|-----------------------|-------------------------------|
| 1-----      | 1.1                 | 8.4/3.7  | 36              | 204                  | 457                   | None.                         |
| 2-----      | 1.3                 | 8.4/4.65 | 36              | 205                  | 457                   | 10% polyamide and delustrant. |
| 3-----      | 1.3                 | 8.4/6.3  | 60              | 206                  | 274                   | 0.1% phenolic antioxidant.    |
| 4-----      | 1.3                 | 7.0/4.65 | 36              | 205                  | 457                   | 10% polyamide and delustrant. |
| 5-----      | 1.55                | 8.4/7.7  | 36              | 205                  | 366                   | None.                         |
| 6-----      | 1.55                | 7.7/4.7  | 24              | 203                  | 655                   | 10% polyamide.                |
| 7-----      | 1.8                 | 8.4/5.1  | 48              | 206                  | 195                   | 10% polyamide and delustrant. |

which has been chain terminated during polymerisation, as for example by the use of hydrogen as chain terminator, and which has a broad molecular weight distribution, may be used as the second component. The proportion of a particular component in the composite filament may be varied between about 1:9 to 9:1 the self-crimping effect obtained over this range being somewhat dependent upon the difference between the Q values for each component. Thus if the Q value difference is high the proportion of the components may differ more from 1:1 than for small Q value differences.

Component polymers may contain up to about 20% by weight of other substances, as for example, stabilising substances, delustrants or pigments or substances conferring an affinity for dyestuffs on the propylene polymers.

Where the term viscosity is referred to herein, in relation to the process of the invention, intrinsic viscosity measured in decalin solution at 135° C. using a viscometer capillary diameter of 0.44 mm. is meant; the units of viscosity being decilitres/gram.

In selecting suitable propylene polymers for use in the preparation of composite filaments according to the invention, we prefer to use polymers which, in addition to having a difference between the Q values of a selected pair of at least about 0.5, also have an intrinsic viscosity of not less than 1.0, as little or no self crimping effect is obtained with polymers of lower viscosity, particularly if the difference in Q value for the pair is low.

The following examples illustrate the invention and the

All percentages are by weight of the polymer composition.

The spun yarns were collected on rigid bobbins and drawn using a heated feed roll, whereon drawing took place, drawing apparatus with a draw roll temperature of 20° C. or 100° C. In all examples except No. 5 a draw ratio of 3.5:1 was applied and in the case of Example 5 a draw ratio of 3.0:1 was applied. The feed 55 roll in all cases was maintained at 55° C.

The properties of the drawn yarns made into 100 cm. hanks and treated as hereinbefore described are given in the following table together with the draw roll temperature used.

| Example No. | Draw roll temp., °C. | Percent crimp at a load of— |                |
|-------------|----------------------|-----------------------------|----------------|
|             |                      | 0.01 mg./denier             | 0.5 mg./denier |
| 1-----      | 20                   | 51                          | 8              |
| 2-----      | 20                   | 64                          | 36             |
| 3-----      | 100                  | 57                          | 24             |
| 4-----      | 100                  | 60                          | 30             |
| 5-----      | 100                  | 56                          | 14             |
| 6-----      | 100                  | 71                          | 63             |
| 7-----      | 20                   | 66                          | 50             |

#### Comparative example A

For comparison a 1.1 composite filament was spun using the apparatus of the foregoing Examples 1-7 and a pair of propylene polymers of Q values 5.9 and 4.65. A 36 hole (0.051 cm. diameter) spinneret maintained at 205° C. was used and the spun yarn was collected on

bobbins at 457 metres/minute. The polymers were of intrinsic viscosity 1.3 and contained 10% of a polyamide to enhance dye affinity. The spun filaments each having a denier of 15 were drawn using a hot feed roll at 55° C. and a cold draw roll with a draw ratio of 3.5:1.

Upon hot relaxation of the drawn yarn no crimp was formed.

#### EXAMPLES 8-14

Composite filaments having varying proportions of the two components in side-by-side relationship were spun and drawn with apparatus as used in Examples 1-7, the proportions of the two components being controlled by varying the rate of supply of the molten components to the spinneret orifices while maintaining a constant spun denier per filament of 15. The propylene polymers used had Q values of 8.4 and 4.65, an intrinsic viscosity of 1.3 and contained 0.5% of calcium stearate and 10% of a polyamide. Spinning was carried out at 205° C. through a 36 hole (0.051 cm. diameter) spinneret the spun filaments being collected at 343 metres/minute and afterwards drawn with a draw ratio of 3.5:1 using feed and draw rolls heated to temperatures of 55° C. and 100° C. respectively. The percentage crimp of the products made in this way are shown in the following table together with the proportions of component polymers used. Component A is that having Q=4.65 and for component B,Q=8.4.

| Example No. | Ratio A:B | Percent crimp at a load of— |                |
|-------------|-----------|-----------------------------|----------------|
|             |           | 0.01 mg./denier             | 0.5 mg./denier |
| 8-----      | 1:1       | 65                          | 30             |
| 9-----      | 2:1       | 60                          | 24             |
| 10-----     | 3:1       | 62                          | 22             |
| 11-----     | 4:1       | 60                          | 16             |
| 12-----     | 2:3       | 54                          | 20             |
| 13-----     | 1:2       | 48                          | 13             |
| 14-----     | 1:3       | 41                          | 11             |

#### Comparative example B

For further comparison a 1:1 composite filament was produced using the apparatus of Examples 1-7 and a pair of propylene polymers having Q values close to the values of the components used in Example 7 but differing in intrinsic viscosity. Thus one component had a Q value of 8.4 and an intrinsic viscosity of 2.1 and the other component had a Q value of 5.2 and an intrinsic viscosity of 1.8. When spun and drawn as in Example 7 this pair of polymers produced a filamentary yarn having a percentage crimp under a load of 0.5 mg./denier of 64%.

What I claim is:

1. A process for the production of self-crimping polypropylene filaments wherein composite filaments having two propylene polymers distributed along the length of the filaments as distinct components in side-by-side or sheath-core relationship are produced by conjugate melt spinning of two propylene polymers followed subsequently by relaxation of tension in the filaments, characterized in that the two polymers have substantially the same intrinsic viscosity, but different molecular weight distributions and wherein the dispersion coefficient, defined as the ratio of weight average molecular weight to number average molecular weight, of at least one of the polymers is at least 6.5.
2. A process according to claim 1 wherein the dispersion coefficients of the component polymers differ by at least 0.5.
3. A process according to claim 1 wherein the component polymers have an intrinsic viscosity of at least 1.0.
4. A process according to claim 1 wherein the ratio of the components is between 1:9 and 9:1.
5. A process according to claim 1 wherein the unrelaxed spun filaments are drawn 2-4 times their original length.
6. A process according to claim 5 wherein the drawing is effected upon a snubbing surface heated to a temperature not greater than 100° C.
7. A process according to claim 5 wherein the drawn filaments are heat treated on a draw roll heated to a temperature up to 100° C.
8. A process according to claim 5 wherein the crimped filaments are stabilised by heat treatment at 100-140° C.

#### References Cited

##### UNITED STATES PATENTS

- |           |         |                       |           |
|-----------|---------|-----------------------|-----------|
| 3,161,914 | 12/1964 | Bloomfield et al. --- | 264—171 X |
| 3,209,402 | 10/1965 | Riley et al. -----    | 18—8      |
| 3,225,534 | 12/1965 | Knope -----           | 57—14     |
| 3,264,390 | 8/1966  | Tanner -----          | 264—171   |

##### FOREIGN PATENTS

- 969,110 9/1964 Great Britain.

JULIUS FROME, *Primary Examiner.*

J. H. WOO, *Assistant Examiner.*